

# UNITED STATES PATENT OFFICE.

WILLIAM S. HOUGHTON, OF BOSTON, MASSACHUSETTS.

## PAVEMENT AND METHOD OF MAKING THE SAME.

No. 888,886.

Specification of Letters Patent.

Patented May 26, 1908.

Application filed September 23, 1907. Serial No. 394,092.

To all whom it may concern:

Be it known that I, WILLIAM S. HOUGHTON, a citizen of the United States, residing at Boston, in the county of Suffolk and State of Massachusetts, have invented a certain new and useful Improvement in Pavements or Roadways and Method of Making the Same, of which the following is a full, clear, and exact specification, reference being had 10 therein to the accompanying drawings.

This invention relates to pavements or roadways and especially to pavements which are monolithic or laid in one course.

Heretofore, it has been customary to lay 15 pavements in courses or layers. The most common type of such pavement comprises three courses, namely, a substratum or foundation, a binder course and an upper layer or wearing surface. The binder course 20 is relied upon, in such cases, to bind the wearing surface to the foundation and is generally made of bituminous or other similar material of strongly adhesive qualities. In other cases, the binder course is dispensed with and a bituminous wearing 25 surface employed, in which event, the adhesive- ness of the wearing course binds it to the foundation. It is necessary to the life of such pavements, however, that the courses 30 or layers should at all times remain firmly bound together; but frequently, owing to the fact that the bituminous binder or the bituminous wearing surface is softened by heat and the adhesion of the wearing sur- 35 face to the underneath layer thereby less- ened or destroyed, the wearing surface, when subjected to the pressure of traffic, slides, rolls or buckles and breaks up. This has been the principal difficulty with pave- 40 ments laid in courses and this defect has never been entirely eradicated.

The object of my invention is to provide a pavement of durable construction which can be laid with facility and economy, and 45 which will not slide, buckle or seam, and I accomplish this purpose by constructing the pavement in one layer which is an integral body or mass, homogeneous in structure.

In the accompanying drawing, which illus- 50 trates the preferred embodiment of my invention, I have shown a vertical cross-sectional view of a portion of a pavement.

Referring to the drawing, 1 represents a curb; 2 broken or crushed stones; and 3

the sand and cement and sand and screen- 55 ings.

In making my pavement, I first prepare a mixture of sand, dry cement and crushed or broken stone, the last mentioned material ranging in size preferably from screenings 60 to two inches in diameter, and constituting about ninety per cent. by weight of said mixture. After the above ingredients have been thoroughly mixed together, they are treated with liquid bitumen, oil or coal tar 65 or liquid asphalt, in such a manner and to such an extent as to coat the particles of sand, stone and cement. This mixture is laid in a solid mass or layer upon the ground which should previously be smoothed to re- 70 ceive it, and then rolled to form a close homogeneous mass. The depth of this layer may vary from four to eight inches to conform to the requirements of the pavement. The liquid bitumen acts as a binding mate- 75 rial to unite the various particles of sand and crushed stone. The amount of liquid bitumen, oil or coal tar or liquid asphalt to be used will depend somewhat upon the size of the stony elements, but enough should be 80 used to coat the particles either partially or entirely.

When the pavement has been thoroughly rolled and compressed, I next mix together dry cement and screenings and spread the 85 mixture over the surface of the pavement in a thin layer. The pavement is then sprinkled with water which washes the mixture of screenings and cement into the voids of the pavement, fills them up, and the cement sets. 90 The water thus sprinkled on the pavement also percolates through the voids and causes the dry cement throughout the pavement which has not been affected by the liquid bitumen, tar or asphalt to set and thus fills 95 up all the voids completely and forms a close and dense mass. If necessary, a second coating of the mixture of screenings and dry cement may be sprinkled on the pavement and treated with water as above described, 100 for the purpose of filling any voids which may not have been entirely closed up by the first application.

In making my pavement, I prefer to use the bitumen, coal tar, asphalt in liquid form 105 because the particles of stone, sand and cement are thereby more easily and efficiently coated and the expense and labor of

providing heating means is dispensed with. In extremely cold weather, it may, however, be necessary to employ heating means but under ordinary conditions, my pavement can 5 be constructed without any heat.

By employing a bituminous substance in liquid form as a binder in addition to the cement, I secure a pavement which is yielding and elastic and therefore less liable to 10 break up or seam when subjected to strain than a pavement where cement alone is used. At the same time by using cement, I secure great strength and wearing qualities.

My invention may also be applied to re- 15 surfacing old macadam roads and is especially adapted to such use owing to the fact that the old materials may be used and a great saving in materials thereby effected. In such a case, I tear off the old macadam, 20 screen out the stone and mix it as previously described. The screenings from the old road are also used in the same manner as heretofore described.

It is to be noted that the wearing surface 25 of my pavement is composed of stony surfaces intermixed with cement surfaces, and is of sufficient roughness to prevent vehicles skidding when passing over it at high speed. Also, since there is no loose material through- 30 out the pavement, it is not subject to the same objections that so largely obtain at the present time with respect to the ordinary macadam or concrete roads. It is a well known fact that the high speed incident to 35 automobile travel causes a strong suction under and to the rear of the automobile as it travels over the road and the suction so generated soon destroys the surface of the road by drawing out the fine particles or 40 dust between the larger stony elements, and leaving large voids which sooner or later cause the surface of the road to be broken up and disintegrated.

Another advantage derived from con- 45 structing my pavement in one homogeneous mass, is that in case of leaks in the gas or water mains in the street, the gas or water cannot affect the pavement. Where roads are constructed in courses or layers, it is fre- 50 quently found that gas or water leaking from the mains forces its way in between the

courses and destroys the road. Where gas gets under the wearing surface it forms a cushion and the wearing surface rolls or waves when used and ultimately breaks up. 55 Water will effect the same final result by washing sand up between the layers.

Since my pavement is all wearing surface, it may be laid in varying thicknesses to suit the use. For example, in a parkway where 60 there is no heavy traffic, it may be laid about four inches deep, which will be found sufficiently strong and durable for such use. For heavy teaming, it should be from six to eight inches in depth. The wearing surface can 65 never be destroyed until the pavement has been worn down to such an extent that the traffic pressure will break it up, and therefore, it is well adapted to long and continuous use. 70

What I claim is:—

1. A pavement, consisting of a single layer or course of a mixture of crushed or broken stone, sand and cement in such proportions as to leave voids, the pieces and fragments 75 of said mixture being coated with bituminous material and compacted and bonded together into a single homogeneous layer or course, the voids in said course being occupied by a cement mixture. 80

2. The process of making a pavement consisting in preparing a mixture of sand, dry cement and crushed or broken stone in such proportions as to leave voids when laid, treating the said mixture with bituminous 85 material in order to coat the fragments and particles in said mixture, laying the treated mixture in a single course, rolling the said course until it is compact, spreading upon the top of said rolled course a layer of sand 90 or screenings and dry cement and then washing the said layer with water into the voids in said course and thereby filling said voids. 95

In witness whereof, I have hereunto set my hand, in the presence of two subscribing witnesses, this the fourth day of September, 1907.

WILLIAM S. HOUGHTON.

Witnesses:

E. F. UNIAC,

CHARLES F. RICHARDSON.